

## UNITED STATES PATENT OFFICE

1,930,145

METHOD FOR MAKING ACETONE SOLUBLE  
CELLULOSE ACETATE WITH ALDEHYDEThomas F. Murray, Jr. and Harry Le B. Gray,  
Rochester, N. Y., assignors to Eastman Kodak  
Company, Rochester, N. Y., a corporation of  
New YorkNo Drawing. Application November 5, 1930  
Serial No. 493,687

15 Claims. (Cl. 260—101)

This invention relates to a process for producing acetone-soluble cellulose acetate, and more particularly to a process in which acetone-soluble cellulose acetate is produced in a single 5 acetylation step, with the aid of an aldehyde.

In the usual procedure for the production of cellulose acetate for use in the arts cellulose is acetylated to a triacetate and subsequently partially deacetylated or "hydrolyzed" until a 10 product is obtained which is soluble in acetone. Since the acetone soluble variety of cellulose acetate was first prepared, attempts have been made to find a method by which it may be made acetone soluble without subsequent hydrolysis. 15 Such a procedure would have an enormous technical value. Because of its saving of time, space, apparatus, chemicals and labor, it would have an economical advantage yet to be estimated.

The present process proposes the use of a substantial amount of an aldehyde, as an agent of addition in the acetylation of the cellulose. It has been previously known to carry out this acetylation in the presence of small amounts of formaldehyde, but the proportion used was not sufficient to produce acetone-soluble cellulose acetate, the formaldehyde being added merely for a stabilizing effect. In addition there are the well known difficulties of working with formaldehyde in any quantity. Also, previously it has not been known 20 that the aldehydes have the function of controlling the acetylation reaction in the manner described, that is, producing acetone-soluble cellulose acetate.

We have found that the addition of acetaldehyde or other appropriate aldehyde to acetic anhydride in the acetylation of cellulose causes the formation of a cellulose derivative which is directly soluble in acetone. The procedure introduces no technical difficulties. Acetaldehyde is cheap and easily available in commercial quantities. Any unused aldehyde can be recovered or easily oxidized to acetic acid.

Specifically, the process is carried out in the following steps:

- 45 1. To about 50 grams of air-dried cotton linters is added a mixture of about 333 cubic centimeters of glacial acetic acid and approximately two cubic centimeters of a catalyst (preferably 95% sulphuric acid and 95% phosphoric acid in the ratio of 1 to 3) and the mixture is allowed to stand at room temperature (23 to 25 degrees C) for about 19 hours or longer. If it is desired to eliminate this step 1, the 19 hours standing is eliminated so that all the materials are mixed together 50 and the acetylation is then carried out, although
- 55 without pre-treatment acetylation does not proceed as readily as with it.
2. The pre-treated cellulose of step 1 may next be treated with a mixture of about 140 cubic centimeters of 85% acetic anhydride and 17 to 18 cubic centimeters of acetaldehyde, the whole being intimately mixed in a vessel in a water bath at a temperature of about 18° C. Stirring is continued and the bath is heated slowly and slightly for from 1 1/2 to 4 hours, after which the rate of heating is increased until a maximum of about 40° C is obtained. Stirring is continued at this temperature for a total acetylation of about 22 hours. To the dope thus obtained may be added 100 to 150 cubic centimeters of acetone to give greater fluidity to the dope, which may then be precipitated in hot water. After washing free of acid and drying, the cellulose derivative may be dissolved in acetone, forming a viscous "dope" which can be utilized in various ways such as by 60 coating into sheets, etc.
- 65 3. Broadly, our invention contemplates the making of acetone-soluble cellulose acetate in one step, namely by acetylation only. This eliminates the necessity for the third, or hydrolyzing, step 70 which has previously been necessary. We have also discovered the broad principle that an aldehyde may be employed to obtain acetone-soluble cellulose acetate in the acetylation step.
- 75 4. As low as 25 cubic centimeters of acet-aldehyde per 100 grams of linters may be employed to obtain a product which is soluble in acetone. While we have found that 35 cubic centimeters per 100 grams of linters is to be preferred, we have also found that 80 to a 100 cubic centimeters per 100 grams of linters is suitable in this process.
- 80 5. It is to be understood that the above specific example is not to limit the process as to the time, temperature and materials used, etc. Thus the time and temperature of pre-treatment may be varied as is well known, a different catalyst may be used in the acetylation process, such for instance as sulphuric acid, and the time and temperature of esterification may be changed somewhat, although it is obvious that after acetone-solubility has been obtained there is no need for further acetylation. Precipitation of the cellulose ester from the "dope" in which it is prepared may be accomplished in other precipitants, if desired, such as a weak acetic acid solution.
- 85 6. In addition to acetaldehyde, other aldehydes such as paraldehyde, formaldehyde, propionic aldehyde and butyric aldehyde have been found suitable for the purpose of this invention.
- 90 7. Other cellulose containing material may be 110

used instead of cotton linters and other acetylation catalysts may be used instead of the phosphoric-sulphuric mixture, as known in the art.

What we claim as our invention and desire 5 to be secured by Letters Patent of the United States is:

1. The process of producing an acetone-soluble cellulose acetate which comprises pre-treating cellulose in concentrated organic acid in the presence of an acetylation catalyst, and acetylating the cellulosic material by adding acetic anhydride and at least 25 c.c. of an aldehyde per hundred grams of cellulose employed.

2. The process of producing an acetone-soluble cellulose acetate which comprises pre-treating cellulose in concentrated organic acid in the presence of an acetylation catalyst, and acetylating the cellulosic material by adding acetic anhydride and at least 25 c.c. of an aldehyde containing a plurality of carbon atoms per hundred grams of cellulose employed.

3. The process of producing an acetone-soluble cellulose acetate which comprises pre-treating cellulose in concentrated acetic acid and an acetylation catalyst, and acetylating the cellulosic material by adding acetic anhydride and at least 25 c.c. of an aldehyde per hundred grams of cellulose employed.

4. The process of producing an acetone-soluble cellulose acetate which comprises acetylating cellulose in the presence of 25-100 c.c. of an aldehyde per 100 grams of cellulosic material present.

5. The process of producing an acetone-soluble cellulose acetate which comprises acetylating cellulose in the presence of 35 c.c. of an aldehyde containing a plurality of carbon atoms per 100 grams of cellulosic material present.

6. The process of producing an acetone-soluble cellulose acetate which comprises acetylating cellulose in the presence of 35 c.c. of acetaldehyde, per 100 grams of cellulosic material present.

7. The process of producing an acetone-soluble cellulose acetate which comprises acetylating cellulose in the presence of 25-100 c.c. of acetylaldehyde per 100 grams of cellulosic material present.

8. The process of producing an acetone-soluble cellulose acetate which comprises acetylating cellulose in the presence of 25-100 c.c. of an aldehyde, containing a plurality of carbon atoms, per 100 grams of cellulosic material present.

9. A process for producing cellulose acetate which comprises acetylating cellulose in acetic acid and acetic anhydride in the presence of a catalyst and at least 25 c.c. of acetaldehyde per hundred grams of cellulose employed.

10. A process for producing cellulose acetate which comprises acetylating cellulose in acetic acid and acetic anhydride in the presence of a catalyst and paraldehyde.

11. A process for producing cellulose acetate which comprises acetylating cellulose with acetic acid and acetic anhydride in the presence of a catalyst and propionic aldehyde.

12. Acetone-soluble cellulose acetate resulting from the acetylation of cellulose in the presence of 25-100 c.c. of an aldehyde per 100 grams of cellulose present.

13. The process which comprises acetylating cellulose in the presence of 25-100 c.c. of an aldehyde per 100 grams of cellulose present until cellulose acetate is produced which is soluble in acetone.

14. Acetone-soluble cellulose acetate resulting from the acetylation of cellulose in the presence of acetaldehyde.

15. The process which comprises acetylating cellulose in the presence of acetaldehyde until cellulose acetate is produced which is soluble in acetone.

HARRY LE B. GRAY.  
THOMAS F. MURRAY, JR.

45

110

50

120

55

125

60

130

65

135

70

140

75

145

150